

H. BRUNSWIG.

METHOD FOR THE DETONATION OF EXPLOSIVES.

APPLICATION FILED AUG. 9, 1911.

1,042,643.

Patented Oct. 29, 1912.



WITNESSES:

Prof. F. Kitchell  
E. E. Hall

INVENTOR

Heinrich Brunswig  
or Frank S. Besser  
ATTORNEY.

# UNITED STATES PATENT OFFICE.

HEINRICH BRUNSWIG, OF STEGLITZ, NEAR BERLIN, GERMANY, ASSIGNOR TO E. I. DU PONT DE NEMOURS POWDER COMPANY, OF WILMINGTON, DELAWARE, A CORPORATION OF NEW JERSEY.

## METHOD FOR THE DETONATION OF EXPLOSIVES.

1,042,643.

Specification of Letters Patent.

Patented Oct. 29, 1912.

Application filed August 9, 1911. Serial No. 643,076.

*To all whom it may concern:*

Be it known that I, HEINRICH BRUNSWIG, a subject of the Emperor of Germany, residing at Steglitz, near Berlin, Germany, have 5 invented a new and useful Improvement in Methods for the Detonation of Explosives, of which the following is a full, clear, and exact description.

The general method of detonating explosive charges comprises a detonating fuse which is either introduced into the blasting 10 powder or passed around or through the cap. A detonating fuse consists in a rod of detonating material compressed within a tube in 15 such a manner that an actual wave of detonation proceeds at a uniform velocity along this fuse, and wherever the fuse is used in this specification, this particular thing is meant. To start such a detonating fuse, the 20 general method of procedure is to have a detonating cap in the end of the same which starts the wave of detonation along the detonating fuse. This detonating fuse differs from the ordinary powder fuse in that in 25 stead of having merely a burning material, in it, it is necessary for it to have a detonating material throughout its length. I have discovered that the action of such detonating fuses is considerably increased if the fuse is 30 detonated on opposite sides of the portion thereof which is in contact with the explosive mass to be detonated. In this case the two detonation waves run toward each other and 35 meet either at the surface or inside of the explosive mass to be detonated and increase the action of the same. This is, for instance, the case when a detonating fuse 100 cm. in length is wound around the explosive in such a manner that the center of the fuse, the 40 stretch from about the 45th to the 55th cm. is in intimate contact with the explosive. I determined by tests the increased initial effect brought about under the preceding condition. The substances to be detonated 45 were pressed bodies made of trinitrotoluol of a density of 1.6. Three series of tests were carried out with three different deto-

nating fuses. The ignition was brought about by means of detonating fuses; the core of the first fuse consisting of trinitrotoluol, 50 that of the second fuse of trinitrobenzol chlorid and that of the third fuse of tetrani-tromethylanilin. The detonation was effected by means of a fulminate of mercury cap No. 8, in one series of experiments simultane- 55 ously on both ends, in the other, for the purpose of comparison, on one end only. It was thus shown that with a double ignition of the fuse a detonation was effected in instances in which with a single ignition a par- 60 tial explosion or no explosion was brought about.

This method can be used for explosive charges of all kinds, for mining operations as well as for military explosives, in burst- 65 ing shells, mines, etc.

In the drawings, the figure is a side view, largely in section, of an apparatus by which my improved process may be carried out.

*a* represents the explosive to be detonated; 70 *b* the casing and *c* the core, of the detonating fuse; *d* the fulminate of mercury; *e* the blasting cap; and *f* the ordinary electric blasting fuse. The point where the two explosive waves meet and produce the stronger 75 effect is indicated by the reference letter *g*.

Having now fully described my invention, what I claim and desire to protect by Letters Patent is:

The improvement in the method of det- 80 onating explosives by means of a detonating fuse, which consists in detonating the fuse from two places in such a manner that the two detonation waves running toward each other meet at the surface or inside of the 85 explosive to be detonated.

In testimony of which invention, I have hereunto set my hand, at Berlin, on this 20th day of July, 1911.

HEINRICH BRUNSWIG.

Witnesses:

WOLDEMAR HAUPT,  
HENRY HASPER.